

## UNITED STATES PATENT OFFICE

FRANK O. WOODRUFF, OF NEWTON, MASSACHUSETTS, ASSIGNEE TO HARRY H. BECKWITH, OF BROOKLINE, MASSACHUSETTS

## MANUFACTURE OF SHOE STIFFENER MATERIAL

No Drawing.

Application filed August 12, 1931. Serial No. 556,614.

The subject of this invention is the manufacture of shoe stiffener material more especially of a character simulating in such important characteristics as density, resiliency, translucency, stiffness, etc., the so-called celluloid type of shoe stiffening materials. An object of the present invention is to make possible the utilization of waste or scrap leathers in the manufacture of the shoe stiffening material of the present invention.

While not limited thereto, my invention will now be described as practised when tanned leather scrap, which is available in large quantities and at very low cost, is used as a raw material. A preferred kind of tanned leather scrap is available in the chrome-tanning industry, wherein the practice is to subject the chrome-tanned kid or other hide to a so-called levelling or skiving operation to reduce the hide on its flesh side to a uniform thickness. The chrome-tanned scrap thus produced is in the form of small fragments or cuttings which are soft and easily disintegrable. In fact, the fragments or cutting contain a considerable amount of water, usually about 50%, since the levelling operation is generally performed on the hides while they are still wet with tanning liquor.

In accordance with the present invention, chrome-tanned fragments or cuttings of the character described are charged into a beater engine or hollander, together with sufficient water to ensure free circulation of the mass.

I have found it desirable to use such scrap while it is still wet with tanning liquor, for when the scrap is once dried out, it becomes tough, horny, and difficultly disintegrable. The beaten mass is then formed into a sheet,

preferably on a papermaking machine. The sheet is treated with ammonia in any suitable state, but it is distinctly desirable that the ammoniation be carried out in the presence of considerable moisture. Thus, the ammoniation may be performed by submerging the dry sheet in ammoniated water; or the sheet may be exposed to an atmosphere of ammonia fumes, with either the sheet in wet condition or with the atmosphere laden with moisture.

When ammonia fumes are employed as the

ammoniating reagent, rather than preliminarily drying the sheet and then remoistening, the sheet may be treated while it is still in the wet condition resulting from formation from aqueous suspension. It is, however, preferable to dry the sheet if the ammoniation is to be performed with ammonia water, as in such case the wet sheet tends to pulp up or disintegrate when submersed in the ammonia water.

I have found that when ammoniation is performed under the proper conditions on a sheet of the character described, it becomes incipiently glutinized and acquires a translucent state. Upon drying the sheet, it becomes dense, resilient and stiff, and closely simulates a sheet of celluloid. Such a sheet is eminently adapted for use in making shoe stiffener parts, such as box toes and counters, for I have found that the sheet can be softened by mere prolonged soaking in water, is mouldable to the desired shape in softened condition, and sets in such shape upon drying. When the sheet is used for the fabrication of counters, the counter blanks may be cut from the sheet immediately after ammoniation and before drying, as the moist, ammoniated sheet has the proper temper for moulding. The moulding of the counter blank is preferably performed with the application of heat, so that the counter may be dried and set in the desired shape while in the mould. One of the advantages possessed by the sheet material of the present invention is that it is slowly combustible and requires only water as a softening agent, whereas celluloid is highly combustible and can be softened only by highly inflammable materials.

A specific example of procedure falling within the purview of the present invention may be about as follows. A beater engine about three-fourths full of water is started running with the knives of the roll close to the bed plate. Chrome-tanned leather scrap of the character hereinbefore described and still wet with about 50% by weight of water is gradually added to the beating engine, while running, so as to avoid clogging under the roll. The beating is continued until the

scrap has been reduced to a uniform pulp suspension characterized by a smooth and more or less slimy feel. A beating period of about two hours may be all that is necessary 5 to ensure a pulp suspension which can be formed into a sheet of uniform texture. The beaten pulp suspension having a consistency of, say, about 5%, is then transferred to a stuff chest wherein it is diluted under agitation with water to a consistency of, say, about 1/4% to 1/2%. The dilute pulp suspension is then passed to a wet machine and formed into a sheet which is wound on the make-up roll to the desired thickness and stripped in 10 wet condition therefrom. I have found it necessary to use a special fabric for removing the layer of pulp from the cylinder mould and transferring it to the make-up roll. Thus, when the usual transfer felt is 15 used, the layer of pulp tends to stick to the felt rather than to the make-up roll. The use of napless toweling cloth or similar woven fabric as the pulp carrier obviates the foregoing difficulty. The wet sheet removed 20 from the make-up roll is then dried, preferably under tension, since otherwise it tends to cockle or warp badly on account of the great shrinkage which takes place during drying. The dry sheet may then be ammoniated by dipping it into a solution made up 25 of, say, equal parts of water and ammonia water of 28% concentration. The sheet should be kept immersed for a period of at least about one hour to effect the desired 30 action. The wet, ammoniated sheet is limp and in this condition can be easily cut into counter blanks and moulded into counters, or cut into box toe blanks which can be kept in moist condition and packaged and shipped in 35 such condition to the shoe factory. On the other hand, the sheet may be cut up into shoe stiffener blanks, which are dry when they reach the shoe factory, but which may be rendered soft and mouldable by soaking 40 in water at the shoe factory.

The ammoniation of the sheet can be performed, as already indicated, with ammonia fumes, in which case the sheet in moist condition as removed from the wet machine may 45 be placed in a chamber filled with ammonia fumes which readily penetrate into and incipiently gelatinize the leather fibers to produce the desired product. When the moist, ammoniated sheet is subjected to a drying 50 operation before cutting into shoe stiffener parts, it is preferable to compact the sheet as by passing it between calender rolls before it is completely dried, as this enhances the density, translucency and horn-like character of the product.

While I do not know precisely what reaction takes place on the sheet of leather fibers when it is subjected in the presence of moisture to the action of ammonia, nevertheless my picture is that the ammonia first

serves to detan the fibers by combining with the chrome tanning agent and then partially or incipiently glutinizes the detanned fibers. The partial glutinization is reflected in the dense, horny, and translucent qualities in the finished product. The detanning action is reflected in the ability of the product to absorb water and become softened thereby. On drying, too, the water-softened product simulates untanned leather in its high shrinkage and warping and in its becoming horn-like. 75

The procedure hereinbefore given may be departed from in certain respects, depending upon the particular scrap leather used, the characteristics desired in the ultimate product, and the amounts of material being handled. Thus, where large-scale operation is practised, the time of beating may be much longer than the two-hour period hereinbefore mentioned, especially when a sheet of comparatively high density, even before ammoniation, is desired. Rather than forming a finished sheet composed entirely of leather, I may produce one which has a reinforcement or backing of fabric. For example, a fabric may be applied to the sheet before or after it is taken off the make-up roll of the cylinder machine, in which case the fabric adheres tenaciously to the sheet without the use of extraneous cementing agents. Rather than forming the sheet on a cylinder machine, the sheet may be made on a Fourdrinier machine, in which case the ammoniation may be performed on a continuous sheet, either before drying or after the sheet is taken off the dry end of the machine. Thus, the continuous wet sheet formed on the wire may be passed through a chamber filled with ammonia fumes before it reaches the drum driers; or the dry sheet coming off the drum driers may be passed through a bath of ammonia water and then redried. The heat applied during drying promotes glutinization and so shortens the time of contact necessary between the ammonia and the sheet. 95

The reinforcement of the sheet may be effected during its formation, by which I mean that the aqueous suspension of leather fibers may be deposited as a layer on a coarsely woven fabric, such as cheesecloth, thereby obviating the step of applying the fabric to a preformed sheet of fibers. 100

It is to be observed that I perform the beating operation on tanned leather fibers and partially or incipiently glutinize the leather fibers only after the formation of the sheet. By so doing, I avoid loss of raw material in the water drained from the paper-making machine, as little material is leached out of the tanned leather during the beating operation. Moreover, the leather fibers can be maintained sufficiently long to permit their interfelting on the paper machine into a porous sheet of considerable strength and tear 115 120 125 130

resistance, even before the sheet is ammoniated. Were the ammonia treatment performed in the beater engine, not only would there be considerable loss of ammonia because a great excess is needed in reacting upon the highly dilute stock in the beater engine, but the glutinized material, being soluble in water, would be lost in considerable amount along with the water removed during sheet formation.

The use of ammonia is of advantage, in that it is a volatile glutinizing agent and effects the desired partial or incipient glutinizing action on the sheet, without tending to disintegrate it. During drying, substantially all of the ammonia is removed, so that the sheet is free from malodors or adulterants which detract from its translucency and horn-like character.

In producing the product of the present invention, it is essential to use only fibrous material upon which ammonia can react. Were cellulose fiber incorporated in substantial amount into the leather furnish, one could not secure a product having the characteristics hereinbefore noted, for cellulose fibers are practically inert with respect to ammonia, and would tend to render the product opaque, as well as to detract from its density, resiliency, and horn-like qualities. When cellulose fiber is used in substantial amount, the product, even after ammoniation, is paper-like in its characteristics. On the other hand, one may use animal fibers, such as goat's or cow's hair, along with the leather, as such fibers are partially glutinized along with the leather during the ammoniating treatment.

The product may be modified somewhat by the use of various agents. Thus, it may be hardened by impregnation with an aqueous solution of sodium silicate, and then drying. It may be permanently softened somewhat by treatment with an aqueous solution of glycerin or so-called fat liquors, e. g., sulfonated castor oil. These treatments may be performed while preserving such qualities as translucency, density, and resiliency in the product, and without deleteriously affecting the ability of the product to be rendered soft and mouldable by mere soaking in water.

I claim:

1. Shoe stiffener material comprising a partially glutinized, prefabricated sheet of water-laid, interfelted animal fibers, said sheet being characterized by its translucency, density, resiliency, and ability to be rendered limp and mouldable by soaking in water and to be set in moulded shape.

2. Shoe stiffener material comprising an ammonia-glutinized, prefabricated water-laid sheet of beaten, chrome-tanned-leather scrap, said sheet being characterized by its translucency, density, resiliency, and ability to be rendered limp and mouldable by soak-

ing in water and to be set in moulded shape.

3. A method which comprises beating animal fiber in the presence of water to produce a uniform aqueous pulp suspension, sheeting the pulp, and ammoniating the sheeted pulp in the presence of water to effect partial glutinization of the fiber.

4. A method which comprises beating animal fiber in the presence of water to produce a uniform aqueous pulp suspension, sheeting the pulp, ammoniating the sheeted pulp in the presence of water to effect a partial glutinization of the fiber, and compacting the partially glutinized sheet.

5. A method which comprises beating chrome-tanned leather scrap in the presence of water to produce a uniform aqueous pulp suspension, sheeting the pulp, and ammoniating the sheeted pulp in the presence of water to effect partial glutinization of the leather fibers.

6. A process which comprises beating in water chrome-tanned leather scrap in substantially the same wet condition as it is derived from hides wet with the tanning liquor to produce a uniform aqueous pulp suspension, sheeting the pulp, ammoniating the sheeted pulp in the presence of water to effect partial glutinization of the leather fiber, and cutting the partially glutinized sheet into shoe stiffener parts.

7. A method which comprises reducing animal fiber in the presence of water to a uniform pulp, sheeting the pulp, partially glutinizing the fibers in situ in said sheet in the presence of water, and drying the sheet.

8. A method which comprises reducing leather stock in the presence of water to a uniform pulp, sheeting the pulp, partially glutinizing the pulped leather fibers in situ in said sheet through the action of water and alkali, and drying the sheet.

In testimony whereof I have affixed my signature.

FRANK O. WOODRUFF. 110

115

120

125

130